# EUROPEAN PATENT SPECIFICATION

(11) **EP 2 985 356 B1**
(45) Date of publication and mention of the grant of the patent: **28.02.2018**
(21) Application number: 15180506.6
(22) Date of filing: 11.08.2015
(51) Int. Cl.: C22C 19/05

(54) **DIE-CASTABLE NICKEL BASED SUPERALLOY COMPOSITION**
NICKELBASIERTE SUPERLEGIERUNGSZUSAMMENSETZUNG FÜR DRUCKGUSS
COMPOSITION DE SUPERALLIAGE À BASE DE NICKEL COULABLE

(30) Priority: 11.08.2014 US 201462035525 P; 11.08.2014 US 201462035526 P
(43) Date of publication of application: 17.02.2016
(73) Proprietor: United Technologies Corporation, Farmington, CT 06032 (US)
(72) Inventor: PANDEY, Awadh, Jupiter, FL Florida 33458 (US)
(74) Representative: de Bresser, Sara Jean

(56) References cited:
- EP-A2- 0 068 628
- WO-A1-00/37695
- US-A1- 2003 177 640
- US-A1- 2007 000 581

## Description

### BACKGROUND

The present disclosure relates to nickel based superalloys and, more particularly, to readily die-castable nickel based superalloys for gas turbine engine components.

Gas turbine engines typically include a compressor section to pressurize airflow, a combustor section to burn a hydrocarbon fuel in the presence of the pressurized air, and a turbine section to extract energy from the resultant combustion gases. Gas path components often include cooling airflows such as external film cooling, internal air impingement, and forced convection, either separately, or in combination to continuously remove thermal energy.

The gas path components, such as nozzles (stationary vanes) and buckets (rotating blades), are typically formed of stainless steel, nickel, and cobalt-base alloys that exhibit desirable mechanical and thermal properties. Nickel based superalloys are of high strength, about 1500 MPa, and increased temperature capability, such as above 700°C. These Nickel Base Supealloys (IN713) are not readily castable via a die casting process as the IN713 alloy breaks apart. EP 0068628 discloses a castable nickel base alloy containing chromium, at least one of molybdenum, tungsten and vanadium, tantalum, columbium (niobium), aluminum, titanium, cobalt, iron, carbon, born and zirconium.

### SUMMARY

A nickel based superalloy according to the present disclosure consists of 4.5-5.5 wt % Tungsten (W), 1.5-2.5 wt % Columbium (Cb), 4.5-5.5 wt % Tantalum (Ta), 0.5-5.0 wt % Titanium (Ti), and 0.5-3.0 wt % Aluminum (Al), and optionally:
(i) 0-0.2 wt % Carbon (C);
(ii) 0-0.35 wt % Manganese (Mn);
(iii) 13-15 wt % Chromium (Cr);
(iv) 3.4-5.5 wt % Molybdenum (Mo);
(v) 0.005-0.015 wt % Boron (B)
(vi) 0.05-0.12 wt % Zirconium (Zr)
(vii) 0-1.0 wt % Iron (Fe); and/or
(viii) 0-0.2 wt % Carbon (C), 0-0.35 wt % Manganese (Mn), 13-15 wt % Chromium (Cr), 0-1.0 wt % Cobalt (Co), 3.4-5.5 wt % Molybdenum (Mo), 0.005-0.015 wt % Boron (B), 0.05-0.12 wt % Zirconium (Zr), 0-1.0 wt % Iron (Fe), 0-0.5 wt % Copper (Cu), 0-0.00003 wt % Bismuth (Bi) and 0-0.0005 wt % Lead (Pb),
with the balance being Nickel (Ni) plus incidental impurities.

A further embodiment of any of the foregoing embodiments of the present disclosure includes a gas turbine engine component of, e.g. comprising, the nickel based super alloy, preferably the die-cast nickel based superalloy.

A further embodiment of any of the foregoing embodiments of the present disclosure includes a gas turbine engine rotor blade of, e.g. comprising, the nickel based super alloy, preferably the die-cast nickel based superalloy.

A further embodiment of any of the foregoing embodiments of the present disclosure includes a gas turbine engine component, e.g. rotor blade, of, e.g. comprising, the nickel based super alloy, preferably the die-cast nickel based superalloy as herein described, the die-cast nickel based superalloy preferably die cast at a cooling rate of at least 56 degrees Celsius per second (10^2 degree F per second).

A further embodiment of any of the foregoing embodiments of the present disclosure includes wherein an average gran size is 6.7 mm (ASTM 3) or smaller.

A further embodiment of any of the foregoing embodiments of the present disclosure includes wherein a degree of elemental segregation is lower than in investment casting.

A nickel based superalloy according to another disclosed non-limiting embodiment of the present disclosure includes 0-0.2 wt % Carbon (C), 0-0.35 wt % Manganese (Mn), 13-15 wt % Chromium (Cr), 0-1.0 wt % Cobalt (Co), 3.4-5.5 wt % Molybdenum (Mo), 4.5-5.5 wt % Tungsten (W), 1.5-2.5 wt % Columbium (Cb), 4.5-5.5 wt % Tantalum (Ta), 0.5-5.0 wt % Titanium (Ti), 0.5-3.0 wt % Aluminum (Al), 0.005-0.015 wt % Boron (B), 0.05-0.12 wt % Zirconium (Zr), 0-1.0 wt % Iron (Fe), 0-0.5 wt % Copper (Cu), 0-0.00003 wt % Bismuth (Bi), 0-0.0005 wt % Lead (Pb), and the balance Nickel (Ni) plus incidental impurities.

A further embodiment of any of the foregoing embodiments of the present disclosure includes a gas turbine engine component, e.g. a rotor blade, of, e.g. comprising, a nickel based superalloy as described above.

A further embodiment of any of the foregoing embodiments of the present disclosure includes a gas turbine engine component, e.g. rotor blade, of a die-cast nickel based superalloy as described above, the die-cast nickel based superalloy preferably die cast at a cooling rate of at least 56 degrees Celsius per second (10^2 degree F per second).

A nickel based superalloy according to another disclosed non-limiting embodiment of the present disclosure includes a die cast nickel based superalloy including a 0-0.2 wt % Carbon (C), 0-0.35 wt % Manganese (Mn), 13-15 wt % Chromium (Cr), 0-1.0 wt % Cobalt (Co), 3.4-5.5 wt % Molybdenum (Mo), 4.5-5.5 wt % Tungsten (W), 1.5-2.5 wt % Columbium (Cb), 4.5-5.5 wt % Tantalum (Ta), 0.5-5.0 wt % Titanium (Ti), 0.5-3.0 wt % Aluminum (Al), 0.005-0.015 wt % Boron (B), 0.05-0.12 wt % Zirconium (Zr), 0-1.0 wt % Iron (Fe), 0-0.5 wt % Copper (Cu), 0-0.00003 wt % Bismuth (Bi), 0-0.0005 wt % Lead (Pb), and the balance Nickel (Ni) plus incidental impurities.

A further embodiment of any of the foregoing embodiments of the present disclosure includes wherein, the die-cast nickel based superalloy die cast at a cooling rate of at least 56 degrees Celsius per second (10^2 degree F per second).

A further embodiment of any of the foregoing embodiments of the present disclosure includes, wherein an average gran size is 6.7 mm (ASTM 3) or smaller.

The foregoing features and elements may be combined in various combinations without exclusivity, unless expressly indicated otherwise. These features and elements as well as the operation of the invention will become more apparent in light of the following description and the accompanying drawings. It should be understood, however, the following description and drawings are intended to be exemplary in nature and non-limiting.

### BRIEF DESCRIPTION OF THE DRAWINGS

Various features will become apparent to those skilled in the art from the following detailed description of the disclosed non-limiting embodiment. The drawings that accompany the detailed description can be briefly described as follows:
Figure 1 is a schematic cross-section of an example gas turbine engine architecture;
Figure 2 is a schematic cross-section of another example gas turbine engine architecture;
Figure 3 is an enlarged schematic cross-section of an engine turbine section; and
Figure 4 is an exploded view of rotor assembly with a single representative turbine blade manufactured of a die castable Nickel Base Superalloy.

### DETAILED DESCRIPTION

Figure 1 schematically illustrates a gas turbine engine 20. The gas turbine engine 20 is disclosed herein as a two-spool turbo fan that generally incorporates a fan section 22, a compressor section 24, a combustor section 26 and a turbine section 28. Alternative engine architectures 200 might include an augmentor section 12, an exhaust duct section 14 and a nozzle section 16 (Figure 2) among other systems or features. The fan section 22 drives air along a bypass flowpath add into the compressor section 24 along a core flowpath, for compression and communication into the combustor section 26, then expansion through the turbine section 28. Although depicted as a turbofan in the disclosed non-limiting embodiment, it should be appreciated that the concepts described herein are not limited to use with turbofans as the teachings may be applied to other types of turbine engine architectures such as turbojets, turboshafts, and three-spool (plus fan) turbofans.

The engine 20 generally includes a low spool 30 and a high spool 32 mounted for rotation about an engine central longitudinal axis A relative to an engine case structure 36 via several bearing compartments 38. The low spool 30 generally includes an inner shaft 40 that interconnects a fan 42, a low pressure compressor ("LPC") 44 and a low pressure turbine ("LPT") 46. The inner shaft 40 drives the fan 42 directly or through a geared architecture 48 to drive the fan 42 at a lower speed than the low spool 30. The high spool 32 includes an outer shaft 50 that interconnects a high pressure compressor ("HPC") 52 and a high pressure turbine ("HPT") 54. A combustor 56 is arranged between the HPC 52 and the HPT 54.

The core airflow is compressed by the LPC 44, then the HPC 52, mixed with the fuel and burned in the combustor 56, then expanded over the HPT 54 and the LPT 46, to rotationally drive the respective low spool 30 and high spool 32 in response to the expansion.

With reference to Figure 3, an enlarged schematic view of a portion of the HPT 54 is shown by way of example; however, other engine sections will also benefit herefrom. A full ring shroud assembly 60 mounted to the engine case structure 36 supports a Blade Outer Air Seal (BOAS) assembly 62 with a multiple of circumferentially distributed BOAS 64 proximate to a rotor assembly 66 (one schematically shown).

The full ring shroud assembly 60 and the BOAS assembly 62 are axially disposed between a forward stationary vane ring 68, and an aft stationary vane ring 70. Each vane ring 68, 70, includes an array of vanes 72, 74 that extend between a respective inner vane platform 76, 78, and an outer vane platform 80, 82. The outer vane platforms 80, 82 are attached to the engine case structure 36.

The rotor assembly 66 includes an array of blades 84 circumferentially disposed around a disk 86. Each blade 84 includes a root 88, a platform 90 and an airfoil 92 (also shown in Figure 4). The blade roots 88 are received within a rim 94 of the disk 86 and the airfoils 92 extend radially outward such that a tip 96 of each airfoil 92 is adjacent to the blade outer air seal (BOAS) assembly 62. The platform 90 separates a gas path side inclusive of the airfoil 92, and a non-gas path side inclusive of the root 88.

The blades 84 are commonly manufactured of a nickel based superalloy, such as IN713 alloy. IN713, however, is not manufacturable via a die casting process as the IN713 alloy breaks apart due to the formation of extremely fine gamma prime precipitates with high volume fraction due to the high cooling rates associated with die casting which provides higher cooling rates than investment casting. In one example die casting provide cooling rates on the order of at least 56 degrees Celsius per second (10^2 degree F per second). The inventors have determined that the relatively high content of aluminum is a primary cause of these castability issues.

The nickel based superalloy according to one disclosed non-limiting embodiment, provides an average gran size that is very fine e.g. 6.7 mm (ASTM 3) or smaller, and the degree of elemental segregation is significantly lower than investment casting due to higher cooling rate in the die casting process. The nickel based superalloy eliminates the potential for cracking when die-cast. This nickel based superalloy contains a relatively lower aluminum wt %, and a higher titanium wt % than that of IN713, as well as contains tungsten, columbium and tantalum to provide a die castable alloy without losing any mechanical properties capability. The tungsten, columbium and tantalum provide strengthening through solid solution, precipitation and carbide formation mechanisms to compensate for the loss in strength from lower aluminum content in the alloy composition. The tungsten forms solid solution with the nickel and also forms MC, M23C6 and M6C carbides (where M is the metal). The columbium forms gamma double prime precipitate which is based on Ni3Nb. The columbium also forms MC and M6C carbides in the alloy composition. The tantalum forms solid solution with nickel and also forms MC carbides in the alloy composition. The tantalum also improves creep strength. The columbium and tantalum facilitates precipitation strengthening through gamma prime formation where these elements can be substituted for aluminum. In addition, higher titanium content in the alloy composition also provides larger volume fraction of gamma prime for strengthening.

The nickel based superalloy according to one disclosed non-limiting embodiment contains a relatively lower wt % Aluminum, such as 0.5-3.0 wt %, and a higher wt % Titanium, such as 0.5-5.0 wt %, as compared to of IN713 that includes 5.5-6.6 wt % Aluminum and 0.5-1.5 wt % Titanium with no Tungsten and no Tantalum.

### EXAMPLE

An example of the nickel based superalloy according to the disclosed non-limiting embodiment, consists of 0-0.2 wt % Carbon (C), 0-0.35 wt % Manganese (Mn), 13-15 wt % Chromium (Cr), 0-1.0 wt % Cobalt (Co), 3.4-5.5 wt % Molybdenum (Mo), 4.5-5.5 wt % Tungsten (W), 1.5-2.5 wt % Columbium (Cb), 4.5-5.5 wt % Tantalum (Ta), 0.5-5.0 wt % Titanium (Ti), 0.5-3.0 wt % Aluminum (Al), 0.005-0.015 wt % Boron (B), 0.05-0.12 wt % Zirconium (Zr), 0-1.0 wt % Iron (Fe), 0-0.5 wt % Copper (Cu), 0-0.00003 wt % Bismuth (Bi), 0-0.0005 wt % Lead (Pb), and the balance Nickel (Ni) plus incidental impurities.

The disclosed nickel based superalloy is readily cast via die casting and has demonstrated good quality without cracking. In addition, the disclosed nickel based superalloy composition has provided at least equivalent or better tensile properties than IN713 alloy. Example components, thus formulated and processed as described above are readily die-cast and exhibit a desirable combination of yield strength, stress rupture properties, environmental resistance, microstructural stability and cost well suited for gas turbine engine applicationsThe use of the terms "a," "an," "the," and similar references in the context of description (especially in the context of the following claims) are to be construed to cover both the singular and the plural, unless otherwise indicated herein or specifically contradicted by context. The modifier "about" used in connection with a quantity is inclusive of the stated value and has the meaning dictated by the context (e.g., it includes the degree of error associated with measurement of the particular quantity). All ranges disclosed herein are inclusive of the endpoints, and the endpoints are independently combinable with each other.

Although the different non-limiting embodiments have specific illustrated components, the embodiments of this invention are not limited to those particular combinations. It is possible to use some of the components or features from any of the non-limiting embodiments in combination with features or components from any of the other non-limiting embodiments.

Although particular step sequences are shown, described, and claimed, it should be understood that steps may be performed in any order, separated or combined unless otherwise indicated and will still benefit from the present disclosure.

## Claims

1. A nickel based superalloy consisting of 4.5-5.5 wt % Tungsten (W), 1.5-2.5 wt % Columbium (Cb), 4.5-5.5 wt % Tantalum (Ta), 0.5-5.0 wt % Titanium (Ti), and 0.5-3.0 wt % Aluminum (Al); and optionally:
(i) 0-0.2 wt % Carbon (C);
(ii) 0-0.35 wt % Manganese (Mn);
(iii) 13-15 wt % Chromium (Cr);
(iv) 3.4-5.5 wt % Molybdenum (Mo);
(v) 0.005-0.015 wt % Boron (B);
(vi) 0.05-0.12 wt % Zirconium (Zr);
(vii) 0-1.0 wt % Iron (Fe); and/or
(viii) 0-0.2 wt % Carbon (C), 0-0.35 wt % Manganese (Mn), 13-15 wt % Chromium (Cr), 0-1.0 wt % Cobalt (Co), 3.4-5.5 wt % Molybdenum (Mo), 0.005-0.015 wt % Boron (B), 0.05-0.12 wt % Zirconium (Zr), 0-1.0 wt % Iron (Fe), 0-0.5 wt % Copper (Cu), 0-0.00003 wt % Bismuth (Bi) and 0-0.0005 wt % Lead (Pb);
with the balance being Nickel (Ni) plus incidental impurities.

2. The nickel based superalloy as claimed in claim 1 consisting of 0-0.2 wt % Carbon (C), 0-0.35 wt % Manganese (Mn), 13-15 wt % Chromium (Cr), 0-1.0 wt % Cobalt (Co), 3.4-5.5 wt % Molybdenum (Mo), 4.5-5.5 wt % Tungsten (W), 1.5-2.5 wt % Columbium (Cb), 4.5-5.5 wt % Tantalum (Ta), 0.5-5.0 wt % Titanium (Ti), 0.5-3.0 wt % Aluminum (Al), 0.005-0.015 wt % Boron (B), 0.05-0.12 wt % Zirconium (Zr), 0-1.0 wt % Iron (Fe), 0-0.5 wt % Copper (Cu), 0-0.00003 wt % Bismuth (Bi) and 0-0.0005 wt % Lead (Pb), with the balance being Nickel (Ni) plus incidental impurities.

3. A gas turbine engine component comprising a nickel based superalloy as claimed in claim 1 or claim 2.

4. A gas turbine engine rotor blade comprising a nickel based superalloy as claimed in claim 1 or claim 2.

5. The gas turbine engine component or rotor blade as recited in claim 3 or claim 4 wherein said superalloy is a die cast superalloy.

6. The gas turbine engine component or rotor blade as recited in claim 5 said die-cast nickel based superalloy die cast at a cooling rate of at least 56 degrees Celsius per second (10^2 degree F per second).

7. The gas turbine engine component or rotor blade as recited in any one of claims 3 to 6, wherein an average gran size is 6.7 mm (ASTM 3) or smaller.

8. The gas turbine engine component or rotor blade as recited in any one of claims 3 to 7, wherein a degree of elemental segregation is lower than in investment casting.

## Patentansprüche

1. Nickelbasierte Superlegierung, bestehend aus 4,5-5,5 Gew.-% Wolfram (W), 1,5-2,5 Gew.-% Niob (Nb), 4,5-5,5 Gew.-% Tantal (Ta), 0,5-5,0 Gew.-% Titan (Ti) und 0,5-3,0 Gew.-% Aluminium (Al); und gegebenenfalls:
(i) 0-0,2 Gew.-% Kohlenstoff (C);
(ii) 0-0,35 Gew.-% Mangan (Mn);
(iii) 13-15 Gew.-% Chrom (Cr);
(iv) 3,4-5,5 Gew.-% Molybdän (Mo);
(v) 0,005-0,015 Gew.-% Bor (B);
(vi) 0,05-0,12 Gew.-% Zirkonium (Zr);
(vii) 0-0,1 Gew.-% Eisen (Fe); und/oder
(viii) 0-0,2 Gew.-% Kohlenstoff (C), 0-0,35 Gew.-% Mangan (Mn), 13-15 Gew.-% Chrom (Cr), 0-1,0 Gew.-% Kobalt, 3,4-5,5 Gew.-% Molybdän (Mo), 0,005-0,015 Gew.-% Bor (B), 0,05-0,12 Gew.-% Zirkonium (Zr), 0-1.0 Gew.-% Eisen (Fe), 0-0,5 Gew.-% Kupfer (Cu), 0-0,00003 Gew.-% Bismut (Bi) und 0-0,0005 Gew.-% Blei (Pb),
wobei der Rest Nickel (Ni) plus zufällige Verunreinigungen ist.

2. Nickelbasierte Superlegierung nach Anspruch 1, bestehend aus 0-0,2 Gew.-% Kohlenstoff (C) ; 0-0,35 Gew.-% Mangan (Mn); 13-15 Gew.-% Chrom (Cr); 0-1,0 Gew.-% Kobalt (Co), 3,4-5,5 Gew.-% Molybdän (Mo), 4,5-5,5 Gew.-% Wolfram (W), 1,5-2,5 Gew.-5 Niob (Nb), 4,5-5,5 Gew.-% Tantal (Ta), 0,5-5,0 Gew.-% Titan (Ti), 0,5-3,0 Gew.-% Aluminium (Al), 0,005-0,015 Gew.-% Bor (B), 0,05-0,12 Gew.-% Zirkonium (Zr), 0-1,0 Gew.-% Eisen (Fe), 0-0,5 Gew.-% Kupfer (Cu), 0-0,00003 Gew.-% Bismut (Bi) und 0-0,0005 Gew.-% Blei (Pb), wobei der Rest Nickel (Ni) plus zufällige Verunreinigungen ist.

3. Komponente eines Gasturbinentriebwerks, umfassend eine nickelbasierte Superlegierung nach Anspruch 1 oder Anspruch 2.

4. Rotorblatt eines Gasturbinentriebwerks, umfassend eine nickelbasierte Superlegierung nach Anspruch 1 oder Anspruch 2.

5. Komponente oder Rotorblatt eines Gasturbinentriebwerks nach Anspruch 3 oder Anspruch 4, wobei die Superlegierung eine Druckgusssuperlegierung ist.

6. Komponente oder Rotorblatt eines Gasturbinentriebwerks nach Anspruch 5, wobei die nickelbasierte Druckgusssuperlegierung bei einer Abkühlgeschwindigkeit von mindestens 56 Grad Celsius pro Sekunde (10² Grad F pro Sekunde) druckgegossen wird.

7. Komponente oder Rotorblatt eines Gasturbinentriebwerks nach einem der Ansprüche 3 bis 6, wobei eine durchschnittliche Korngröße 6,7 mm (ASTM3) oder kleiner beträgt.

8. Komponente oder Rotorblatt eines Gasturbinentriebwerks nach einem der Ansprüche 3 bis 7, wobei ein Grad an Elementtrennung niedriger ist als beim Feinguss.

## Revendications

1. Superalliage à base de nickel constitué de 4,5 à 5,5 % en poids de tungstène (W), 1,5 à 2,5 % en poids de Columbium (Cb), 4,5 à 5,5 % en poids de tantale (Ta), 0,5 à 5,0 % en poids de titane (Ti) et 0,5 à 3,0 % en poids d'aluminium (Al) ; et éventuellement :
(i) 0 à 0,2 % en poids de carbone (C) ;
(ii) 0 à 0,35 % en poids de manganèse (Mn) ;
(iii) 13 à 15 % en poids de chrome (Cr) ;
(iv) 3,4 à 5,5 % en poids de molybdène (Mo) ;
(v) 0,005 à 0,015 % en poids de bore (B) ;
(vi) 0,05 à 0,12 % en poids de zirconium (Zr) ;
(vii) 0 à 1,0 % en poids de fer (Fe) ; et/ou
(viii) 0 à 0,2 % en poids de carbone (C), 0 à 0,35 % en poids de manganèse (Mn), 13 à 15 % en poids de chrome (Cr), 0 à 1,0 % en poids de cobalt (Co), 3,4 à 5,5 % en poids de molybdène (Mo), 0,005 à 0,015 % en poids de bore (B), 0,05 à 0,12 % en poids de zirconium (Zr), 0 à 1,0 % en poids de fer (Fe), 0 à 0,5 % en poids de cuivre (Cu), 0 à 0,00003 % en poids de bismuth (Bi) et 0 à 0,0005 % en poids de plomb (Pb) ;
le reste étant du nickel (Ni) plus des impuretés accidentelles.

2. Superalliage à base de nickel selon la revendication 1 constitué de 0 à 0,2 % en poids de carbone (C), 0 à 0,35 % en poids de manganèse (Mn), 13 à 15 % en poids de chrome (Cr), 0 à 1,0 % en poids de cobalt (Co), 3,4 à 5,5 % en poids de molybdène (Mo), 4,5 à 5,5 % en poids de tungstène (W), 1,5 à 2,5 % en poids de columbium (Cb), 4,5 à 5,5 % en poids de tantale (Ta), 0,5 à 5,0 % en poids de titane (Ti), 0,5 à 3,0 % en poids d'aluminium (Al), 0,005 à 0,015 % en poids de bore (B), 0,05 à 0,12 % en poids de zirconium (Zr), 0 à 1,0 % en poids de fer (Fe), 0 à 0,5% en poids de cuivre (Cu), 0 à 0,00003 % en poids de bismuth (Bi) et 0 à 0,0005 % en poids de plomb (Pb), le reste étant du nickel (Ni) plus des impuretés accidentelles.

3. Composant de moteur de turbine à gaz comprenant un superalliage à base de nickel selon la revendication 1 ou la revendication 2.

4. Pale de rotor de moteur à turbine à gaz comprenant un superalliage à base de nickel selon la revendication 1 ou la revendication 2.

5. Composant de moteur à turbine à gaz ou pale de rotor selon la revendication 3 ou la revendication 4, dans lequel/laquelle ledit superalliage est un superalliage moulé sous pression.

6. Composant de moteur à turbine à gaz ou pale de rotor selon la revendication 5, ledit superalliage à base de nickel moulé sous pression étant moulé sous pression à une vitesse de refroidissement d'au moins 56 degrés Celsius par seconde (10^2 degré F par seconde).

7. Composant de moteur de turbine à gaz ou pale de rotor selon l'une quelconque des revendications 3 à 6, dans lequel une taille de grain moyenne est de 6,7 mm (ASTM3) ou plus petite.

8. Composant de moteur de turbine à gaz ou pale de rotor selon l'une quelconque des revendications 3 à 7, dans lequel un degré de séparation élémentaire est pslus faible que dans un moulage de précision.
